

## UNITED STATES PATENT OFFICE

2,583,399

## CORROSION PREVENTION METHOD

Aaron Wachter, Oakland, Calif., and Wilfrid W. Newschwander, Ellensburg, Wash., assignors to Shell Development Company, Emeryville, Calif., a corporation of Delaware

No Drawing. Application March 5, 1951,  
Serial No. 214,032

11 Claims. (Cl. 252—8.55)

1

This invention relates to a method of corrosion-inhibition of a ferruginous material, e. g., steel, while in contact with an agitated fluid system of liquid or liquefied phases and an atmosphere of aqueous carbonic acid and/or carbon dioxide. More particularly, the invention applies to corrosion-prevention of metal equipment normally used in operating gas-condensate light gasoline wells, whereby such corrosion-prevention is effected during the conventional operation of these wells.

In recent years, the problem of preventing corrosion of ferruginous materials, e. g., steel, in the above-described systems as indicated above has been technically noted as very serious. No satisfactory method is known for preventing corrosion of tubing in operating wells under corrosive conditions indicated above.

It is an object of the present invention to provide an inexpensive and industrially feasible method of corrosion-inhibition of ferruginous metals in a system in which an agitated flowing mixture of non-oxidizing gases, a liquefied hydrocarbon phase and an aqueous carbonic acid phase come in contact with such ferruginous metal. It is another object to overcome the disadvantages of prior art practices peculiar to corrosion-inhibition applied in operation of gas-condensate wells. A further object is to provide an inexpensive and industrially feasible corrosion-inhibition treatment of iron-containing metals, e. g., steel, contacting the above-specified system as it occurs in the case of an operating gas-condensate well.

It has now been discovered that corrosion which is caused by contact of ferruginous metal with a system of non-oxidizing gases and an agitated flowing mixture of a liquefied hydrocarbon phase and an aqueous carbonic acid phase, can be inhibited by introducing (continuously or intermittently) into this system a minor but corrosion-inhibiting amount of a high molecular weight oil-soluble organic sulfonate salt.

Described more specifically, it has been found that corrosion of iron-containing metal tubing and well-head fittings in a flowing gas-condensate well containing water and carbon dioxide is inhibited substantially by mixing with the fluid mixture in the well a salt of a high molecular weight oil-soluble sulfonic acid, and particularly in the case of those operating gas condensate wells wherein there is a liquefied hydrocarbon phase as well as a liquid water phase.

The liquefied hydrocarbon phase in gas-con-

2

densate wells normally comprises mixtures of liquid methane, ethane, propane, butane and heavier hydrocarbon condensates up to and including light gasolines having up to about eight carbon atoms. Normally gaseous hydrocarbons are partly liquefied in the well because of the pressures ordinarily existing therein. A typical gas-condensate well produces between twenty and thirty barrels of a liquefied hydrocarbon phase per million cubic feet of gas (MMCF), at a typical well-head temperature and pressure. The temperatures at the bottom of the well usually range from about 85° C. to about 125° C., average temperatures at the well-head being usually in the range from about 45° C. to about 80° C. Pressures in a condensate well usually range from about 1,000 to about 7,000 pounds per square inch absolute. A typical well may have a bottom-hole pressure of about 2,700 p. s. i. a. and a flowing tubing pressure of about 2,000 p. s. i. a. The pressure increases the ratio of gaseous carbon dioxide (present in condensate wells) which will dissolve in the aqueous phase also present therein. At well-head conditions there is usually a range from about seven to about twenty gallons or higher of liquid water per MMCF of gas produced. This liquid water phase dissolves carbon dioxide thus providing the aqueous carbonic acid phase. The latter usually has a pH value ranging from about 3.3 to about a pH of 5.5. This aqueous phase may also contain sodium chloride and other electrolytes, the usual amounts of which are well known to the art. Aqueous carbonic acid phase mixed with agitated liquefied hydrocarbon phase and gases is usually distributed throughout the flowing system of the well.

The sulfonate salts to be employed in the practice of this invention should have a molecular weight of at least 400 and should not exceed about 1500; preferably the molecular weight range should be from about 400 to about 880. In order to ensure oil-solubility, the sulfonate salt should have an oleophilic residue or radical attached to the sulfonate nucleus, preferably comprising at least one hydrocarbon radical having about 16 or more carbon atoms. The oleophilic radical or residue preferably comprises mono- or poly-aromatic and/or naphthenic ring radicals which are alkylated; however, it may be a saturated, or olefinic aliphatic hydrocarbon radical. Any one hydrocarbon radical in the sulfonate salt should not contain a hydrocarbon radical which is longer than an approximately thirty-carbon 55 straight-chain radical, and the total carbon con-

tent of the sulfonate salts employed should not be more than approximately ninety carbon atoms.

Although any salt (metallic or non-metallic) of an oil-soluble sulfonate as described above may be used, it has been found that the above-specified corrosion-inhibition of steel is particularly achieved by introducing into the system an oil-soluble organic sulfonate salt of a base selected from the inorganic group of basic cations made up of sodium, potassium, lithium, calcium, strontium, barium and ammonium ions, and from the organic group of basic cations made up of organo-nitrogen base ions such as those of the amines, quaternary ammonium ions and the heterocyclic nitrogenous basic ions. Of these basic cations used to form the sulfonate salt, the strong base metal cations of the type of alkali and alkaline earth metal cations are preferred; however, in many cases, the salts of organo-nitrogen bases and the appropriate sulfonic acids have been found to be eminently useful.

The oil-soluble sulfonates of this invention may contain two and even three sulfonate salt groups so long as they are substantially concentrated toward one end or in one anterior portion of the agent molecule and sufficient oil-solubility of the molecule as a whole is present. Preferably, the number of sulfonate groups per molecule is limited to no more than two.

Particularly significant corrosion-prevention in practice of the invention has been obtained with oil-soluble mono- and di-sulfonate salts at concentrations below 0.1 wt. %, as low as 0.001 wt. % and even lower, based on the liquefied hydrocarbon phase. Amounts up to and even more than 1% may be used with benefit if the economics permit it.

By an oil-soluble organic residue in the present agents is meant any oil-solubilizing and substantially water-insolubilizing organic radical containing, or consisting of at least sixteen carbon atoms; preferably it is composed of alkylated aryl or alicyclic rings or heterocyclic rings; it may be less desirably an alkyl group. As an aryl containing oil-solubilizing radical there may be used a benzene or naphthalene ring attached to one or more alkyl groups, wherein one of the latter may serve as an alkylene group, attaching the residue to the sulfonate salt group. The term "aliphatic side-chain" as used herein means a side-chain which is an alkyl, cycloalkyl or mixed alkyl-cycloalkyl radical and which may contain unsaturated linkages.

Hetero-atoms such as oxygen, sulfur, or nitrogen may be present in, or provide interconnecting links in the organic residue connected to the one or more sulfonate salt groups so long as the oil-solubility of the molecule as a whole is retained and the direction of polarity afforded by the sulfonate group is retained.

An oil-soluble sulfonate salt for the present invention may be prepared by neutralization of an oil-soluble sulfonic acid. The "oil-soluble" sulfonic acids are hydrocarbon sulfonic acids (which may contain heterogroups) having a solubility in a lubricating mineral oil of SAE 30 grade of at least approximately 0.1 wt. % at 25° C. Particularly effective for the purpose of the invention are those sulfonates which have an oil-solubility of about 1 wt. % up to about 5 wt. % and even higher. The solubility may be as high as 50 wt. % or higher in a lubricating oil or in a diesel oil. Some of these oil-soluble sulfonic acids may also be partially soluble in water; how-

ever, the present sulfonic acids or their salts do not include those salts which are miscible with water in all proportions. Solubility of many of the present agents in both oils and water results from their having intra-molecularly both a strong water-solubilizing radical and a strong oil-solubilizing radical (or radicals).

The so-called mahogany acids (oil-soluble petroleum sulfonic acids) yield salts useful as the agents in this invention. The mahogany acids include particularly the oil-soluble aromatic sulfonic acids from petroleum. Many of the aromatic sulfonic acids from petroleum have cycloalkyl (i. e., naphthenic) groups in the side-chain(s) attached to the benzene ring. The mahogany acids also include non-aromatic sulfonic acids produced in conventional sulfuric acid refining of lubricating oil distillates and from the industrial use of fuming sulfuric acid in the manufacture of petrolatum. The industrial production of oil-soluble mahogany sulfonates from petroleum is well understood in the art and described in the literature.

Non-aromatic long-chain paraffinic sulfonates which are effective agents in the practice of this invention, may also be prepared by other well known methods, such as may be represented by the equation:



where R is a long-chain hydrocarbon residue. The thus produced alkyl-sulfonyl chlorides upon saponification give desired metal sulfonate salts. Suitable long-chain sulfonates may also be produced by well-known Strecker reactions in which sodium, potassium or ammonium sulfite are reacted with a long-chain organic chloride. Some suitable sulfonates produced by this method are:



A preferred class of sulfonate salts for the present invention are those derived from mono-sulfonic aromatic acids having alkyl and/or cycloalkyl radicals attached to the aromatic ring, and a molecular weight of at least approximately 400. Of particular utility are such sulfonate salts having a molecular weight of about 450 to about 650, so long as the aromatic-sulfonate nucleus therein has a hydrocarbon chain attached thereto having not more than about 30 carbon atoms; preferably, the sulfonate molecule contains a total of not more than about 65 carbon atoms. Of these petroleum-derived sulfonates, the substantially water-insoluble calcium salts thereof are particularly valuable for the purpose of this invention. Those sulfonates which contain on the average at least one aromatic nucleus and at least one naphthenic group per molecule, as obtained from a naphthenic-aromatic oil are especially effective.

Particularly preferred examples of sulfonate salts as agents in the present invention are:



octadecylbenzene sulfonate, octadecyltetralinsulfonate, disodium octadecyltetralindisulfonate, etc. The disodium octadecyltetralindisulfonate exhibits prevention of steel corrosion when tested even at as low a concentration as 0.03 to 0.01 wt.% (based on the liquefied hydrocarbon) in a carbonic acid phase-light gasoline phase agitated system.

In the case of the amine or quaternary ammonium base sulfonates, the amine or quaternary ammonium residue may be short, or it may have a long organic residue which may be the same or substantially similar to the organic residue attached to the sulfur in the sulfonate portion of the salt. The presence of an oil-solubilizing organic group, particularly of a hydrocarbon radical of 16 or more carbon atoms in the nitrogen base residue, surprisingly enough does not substantially detract from the present corrosion-inhibiting effect of the sulfonate salts even though the ratio of the sulfonate nucleus to total molecular weight is greatly decreased. In general, the same oil-soluble sulfonic acids as used in the sulfonates described above may be coupled with organic N-containing bases to form the corresponding N-base sulfonates. Suitable amines for forming the salts are the primary, secondary and tertiary amines. Among these, dimethyl amine, diisopropyl amine, ethyl amine, trimethyl amine, cyclohexyl amine and similar amines are preferred. Illustrative long-chain amines are: lauryl amine, stearyl amine, etc. Illustrative examples of suitable heterocyclic nitrogenous bases are: pyridines, oxazoles, oxazolines, oxazines, diazoles, pyrazoles, pyridazines, piperidines, etc., any one of which may have attached thereto a long chain such as dodecyl, stearyl, etc. The substituted oxazolines, particularly the 2-hydrocarbyl substituted oxazolines, are very effective. The molecular weight of the salt as a whole may go as high as 1500, but the molecular weight should preferably not go above 880.

Illustrative examples of suitable quaternary ammonium bases are: trimethyl benzyl ammonium hydroxide, dimethyl benzyl cetyl ammonium hydroxide, stearyl triethyl ammonium hydroxide, etc.

It is not known just how the present class of inhibitors act to prevent corrosion of steel under the conditions employed in the present invention. Suffice it to say that they have been found to act effectively. This is surprising in view of the turbulence of flow in the system and the low concentrations of inhibitor (less than about 1 wt. %, based on the liquefied hydrocarbon phase) which are effective relative to the much higher concentrations of carbonic acid and other dispersing components in the system. Also, these inhibitors are soluble in the liquefied hydrocarbon phase; so it would seem that they would be dissolved and swept away by the turbulent

flow of this phase, leaving the surface of the metal open to attack by the swiftly churning aqueous carbonic acid present.

The present inhibitors function in the specified system without the necessity of any added free bases such as ammonia, amines, organic hydroxides, inorganic hydroxides, etc. Although free bases may be added to or be present in the system, so far as is known, the inhibitors of the present invention act independently of free bases. When free bases are added to gas-condensate wells, a deleterious effect is brought about due to the rise in the pH value of the aqueous phase to a point that calcium or magnesium ions normally present exceed their solubility product with inorganic salt-anions present and precipitate as salts. The latter causes obstructions or stopages in the wells. On the other hand, the present inhibitors function without substantially changing the pH of the system in gas-condensate wells or the like.

The present agents may be introduced into distillate (condensate) wells in various ways. For example, tubing of relatively small diameter may be run down the center of the production tube of such a well to approximately the bottom end thereof, and a solution of the present agent(s) may be pumped through the small diameter tubing so as to enter the well stream near the bottom of the well tube; the rising turbulent flow will then carry the injected agent up through the tube. Obviously, the corrosion inhibitors may be added or introduced into the wells by other means or methods depending, in part, on whether the wells are operated through the casings or through tubing disposed in such casings. Also, it is clear that the inhibitors may be introduced into the top of the well and allowed to flow down, or may be forced to any given point or points in the well, at which the inhibitor then can come in contact with the turbulent up-flowing fluid mixture which, as stated, would cause metal corrosion but for the presence of the corrosion inhibitors of this invention.

The employment of the present agents is best effected by having them in solution in a liquid hydrocarbon readily miscible with the liquefied hydrocarbon phase of the well system, and then introducing the hydrocarbon solution of the agent or agents to a condensate well as above-described. Any organic solvent which is substantially non-reactive with the agent(s) under the conditions employed, (e.g., such solvents as esters, alcohols, ketones, etc.); may be used for preparing an inhibitor solution, although it is preferable to employ light gasolines or normally liquid or liquefied condensates from the well that is to be treated. In the alternative, a suitable crude oil or crude oil fraction (whether refined or not) is also efficacious as a means of forming a fluid solution which can be flowed or forced into these condensate wells. In some cases it is advantageous to use a more or less concentrated solution or dispersion (as up to about 50 wt. % of the agent(s)) in a suitable fluid medium such as a diesel oil. The amount of solvent in the inhibitor solution is so small, relative to the volume of liquid in the system treated therewith, that it does not materially affect the normal operation of the well.

The agents of the present invention employed in the operation of light gasoline gas-condensate wells have not caused emulsion troubles. However, in cases where undesirable emulsification is produced for one reason or another, this can

be prevented or inhibited by the addition of a wide variety of emulsion-breakers or demulsifiers, such as 2-ethyl hexanol, lauryl alcohol, octadecanol, high and low molecular weight silicones and organic silicates.

For purposes of further illustration, reference will now be made to the following examples, it being understood that there is no intention of being limited necessarily to the specific conditions disclosed therein. In these examples steel plates (3/8 inch width, 5 1/8 inch length sandblasted cold-rolled steel strips) were placed in oil-container pressure-bottles containing 10 g. of a water solution having 0.05 wt. per cent of sodium chloride and 50 g. of iso-octane containing in some cases a hydrocarbon-soluble additive of the present invention. In certain cases, the water phase also contained 0.05 wt. per cent of acetic acid. The concentration of the hydrocarbon soluble additive was based upon the iso-octane (hydrocarbon) content. The contents of each bottle were then saturated with carbon dioxide gas as follows: Air was displaced by passing a carbon dioxide to the bottom of each bottle for approximately 15 minutes. Then, the pH value of the aqueous phase was measured. Carbon dioxide was again passed in as previously, for about 5 minutes, and the operation repeated until the pH of the aqueous phase was constant. The prepared bottles were then tightly closed and the stoppers wired on to withstand the pressure developed at elevated temperatures. The bottles were then rotated end-over-end at 60 R. P. M. at a temperature of approximately 65° C. for a period ranging from 18 to 24 hours. At the end of this time the corrosion rates were measured for each steel plate. The results obtained from following the above-described technique are given below.

#### Example I

A series of steel plates were subjected to the above treatment in a container having 50 grams of iso-octane and 10 grams of water, the latter containing 0.05 wt. per cent of sodium chloride. No corrosion inhibitor was present. An analysis of the thus treated plates showed that the average corrosion rate was about 21.0 mils per year.

In another series, the steel plates were likewise treated except that the water phase, in addition to the sodium chloride also contained 0.05 wt. per cent of acetic acid (based on the water). In this case the average corrosion rate was found to be 39.0 mils per year.

#### Example II

Steel plates of the above type were treated in the same manner in the absence of acetic acid but in the presence of a reaction product formed by the interaction of equimolar amounts of 2-(heptadecen-8-yl)-4-methyl-4-(1-hydroxypropyl)-2-oxazoline and of monobasic oil-soluble petroleum sulfonate acids, this reaction product being employed in concentrations of 0.005 wt.% and 0.01 wt.%, as calculated on the iso-octane present in the mixture. The corrosion rates were found to be 0.9 and 0.5 mil per year, respectively.

When the above test was repeated with the same additive and in the presence of 0.05 wt.% of acetic acid, the corrosion rate was about 1.3 mils per year.

#### Example III

When the steel plates were treated as above described, in the absence of acetic acid, but in

the presence of an additive prepared from a mixture of oil-soluble substituted oxazoline compounds, sold under the trade name of "Alkaterge O" and a corresponding mol. equivalent of oil-soluble petroleum sulfonic acids employed to form the additive used in Example II, which additive was used in concentrations of 0.005%, 0.01% and 0.03% (as calculated on the iso-octane content), the corrosion rates were 1.7, 0.5 and 1.2 mils per year, respectively.

#### Example IV

When the steel plates were treated as described above, in the absence of acetic acid, but in the presence of an additive composition composed of a low viscosity index lubricating oil containing 2.5 wt.% of oil-soluble sodium mahogany petroleum sulfonates, 2.5 wt.% of oleic acid and 0.5 wt.% of sodium oleate, and when this composition was used in concentrations of 0.0011%, 0.0023% and 0.014% (as calculated on the sodium petroleum sulfonates content relative to the liquid iso-octane present) the corrosion rates were 1.8, 1.6 and 1.5 mils per year, respectively.

#### Example V

When the steel plates were treated as above described in the presence of oil-soluble sodium mahogany petroleum sulfonates employed in concentrations of 0.005%, 0.01% and 0.06%, based on the iso-octane, the corrosion rates were 2.0, 1.5 and 0.7 mils per year, respectively.

#### Example VI

When the steel plates were treated as above described, in the presence of acetic acid, but in the presence of oil-soluble calcium mahogany petroleum sulfates employed in concentrations of 0.005%, 0.01% and 0.03% (based on the iso-octane), the corrosion rates were 0.5, 1.8 and 1.2 mils per year, respectively. When using this additive in a concentration of 0.01%, and when 0.05% of acetic acid were present, the corrosion rate was found to be 2 mils per year.

#### Example VII

When the steel plates were treated as described above, in the absence of acetic acid, but in the presence of an additive composed of 3.2 wt.% of oil-soluble sodium mahogany petroleum sulfonates dissolved in a blend of approximately 22 wt.% of a low viscosity index lubricating oil and about 70 wt.% of a mineral spirits petroleum distillate (the remainder including about 22 wt.% of ammonium ricinoleate), about 0.8 wt.% of n-butanol, and about 1.1 wt.% of lard oil, it was found that by using this additive in concentrations (calculated on the ratio of petroleum sulfonates to the liquid iso-octane) of 0.004%, 0.012% and 0.016%, the corrosion rates were 0.2, 0.3 and 0.3 mils per year, respectively; in similar runs in the presence of acetic acid, the corrosion rates were 3.0, 1.2 and 1.9 mils per year, respectively.

#### Example VIII

When steel plates were treated as described above, in the absence of acetic acid, but in the presence of an additive composed essentially of one part by weight of oil-soluble sodium petroleum hydrocarbon sulfonates, and nine parts by weight of glyceryl monooleate (which additive was used in the form of a 5% solution in a low viscosity index neutral lubricating oil), and when its concentrations (based solely on the sodium hydrocarbon sulfonates relative to the liquid iso-

octane) were 0.0022% and 0.0033%, the corrosion rates were found to be 2.0 and 1.8 mils per year, respectively.

*Example IX*

In tests conducted in gas-condensate wells in the Sheridan field in Texas, 6 pounds per day of a 50-50 mixture of glyceryl monooleate and sodium petroleum mahogany sulfonate were injected into a well producing at an average production rate of about 6.0 million cubic feet per day. The corrosion rate was determined by means of measured weight losses of 0.1 inch thick, 5 inch diameter plates having a 1 inch diameter orifice in the center, said plate being at a flanged joint upstream from the wellhead choke. After 89 days of injection it was found that the corrosion rate had been reduced to less than 1 mil per day.

*Example X*

When the test of Example V is repeated using an equivalent amount of the barium salt of a sulfonated wax phenol, a similarly substantial reduction in corrosion is obtained.

*Example XI*

When the procedure of Example IV is repeated, but using a sodium dialkylnaphthalene sulfonate, or the cyclohexylammonium salt of sulfonated sperm oil, instead of the calcium petroleum mahogany sulfonates, similar results are obtained.

The introduction of a number of the above described sulfonate salt additives into well streams of gas-condensate wells in the above indicated concentrations and also in higher practicable amounts as described according to this invention in the above specification, have resulted in decrease in the iron content of the effluent water and in a significantly decreased corrosion rate of steel coupons placed within the well stream.

The process of the present invention is also applicable to treatment of wells in which the hydrocarbon phase, under the operating conditions, is substantially solely in the gaseous state.

This application is a continuation-in-part of application Serial No. 764,593, filed July 29, 1947, now abandoned.

We claim as our invention:

1. The method of treating a hydrocarbon-containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and seven thousand pounds per square inch absolute, comes in contact with corrodible well parts, which method includes the step of mixing with said system an amount of below approximately one weight per cent and above approximately 0.0001 weight per cent of the liquid hydrocarbon phase contacted, of an oil-soluble sodium petroleum mahogany sulfonate salt having a molecular weight between about 450 and about 650, said salt having an oleophilic residue containing at least about 16 carbon atoms.

2. The method of treating a hydrocarbon-containing system in its natural state in a well for the purpose of inhibiting corrosion by aqueous carbonic acid of well metal parts, said system comprising a non-oxidizing gas phase, a lique-

fied normally gaseous hydrocarbon phase and a minor amount of aqueous carbonic acid, which system in a state of agitated flow at temperature of between about 45° C. and about 125° C. and under a pressure of between about fifteen and about seven thousand pounds per square inch absolute, comes in contact with corrodible well parts, which method includes the step of mixing with said system an amount of below approximately 1 weight per cent and above approximately 0.0001 weight per cent of the liquid hydrocarbon phase contacted, of an oil-soluble alkali metal petroleum mahogany sulfonate salt having a molecular weight between about 450 and about 650, said salt having an oleophilic residue containing at least about 16 carbon atoms.

3. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and about seven thousand pounds per square inch absolute, comes in contact with corrodible well parts, which method includes the step of mixing with said system an amount of below approximately one weight per cent and above approximately 0.0001 weight per cent of the liquid hydrocarbon phase contacted, of an oil-soluble alkali metal petroleum mahogany sulfonate salt having a molecular weight between about 400 and about 880, said salt having an oleophilic residue containing at least about 16 carbon atoms.

4. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and about seven thousand pounds per square inch absolute, comes in contact with corrodible well parts, which method includes the step of mixing with said system an amount of below approximately one weight per cent and above approximately 0.0001 weight per cent of the liquid hydrocarbon phase contacted, of an oil-soluble alkaline earth metal petroleum mahogany sulfonate salt having a molecular weight between about 400 and about 800, said salt having an oleophilic residue containing at least about 16 carbon atoms.

5. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and about seven thousand pounds per square inch absolute, comes in contact with corrodible well parts, which method includes the step of mixing with said system an amount of below approximately one weight per cent and above approximately 0.0001 weight per cent of the liquid hydrocarbon phase

11

contacted, of an oil-soluble base metal petroleum mahogany sulfonate salt having a molecular weight between about 400 and about 880, said salt having an oleophilic residue containing at least about 16 carbon atoms.

6. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and about seven thousand pounds per square inch absolute, comes in contact with corrodible well parts, which method includes the step of mixing with said system an amount of below approximately one weight per cent and above approximately 0.0001 weight per cent of an oil-soluble sodium salt of an aryl sulfonic acid having a molecular weight between about 450 and about 650, said salt having an oleophilic residue containing at least about 16 carbon atoms.

18 carbon atoms.

7. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and about seven thousand pounds per square inch absolute, comes in contact with corrodible well parts, which method includes the step of mixing with said system an amount of below approximately one weight per cent and above approximately 0.0001 weight per cent of an oil-soluble sodium salt of an organic sulfonic acid having a molecular weight between about 400 and about 880, said salt having an oleophilic residue containing at least about 16 carbon atoms.

8. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow at a temperature of between about 45° C. and about 125° C. and under a pressure of between about fifteen and about seven thousand pounds per square inch absolute, comes in contact with corrodible well parts, which method includes the step of mixing with said system an amount of below approximately one weight per cent and above approximately 0.0001 weight per cent of an oil-soluble salt of an organic sulfonic acid having a molecular weight between about 450 and 880, said salt having an oleophilic residue containing at least about 16 carbon atoms.

9. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor

12

amount of aqueous carbonic acid, which system in a state of agitated flow at a temperature of between about 45° C. and about 125° C. and under a pressure of between about fifteen and about seven thousand pounds per square inch absolute, comes in contact with corrodible well parts, which method includes the step of mixing with said system an amount of below approximately one weight per cent and above approximately 0.0001, weight per cent of an oil-soluble oxazoline salt of an aryl sulfonic acid having a molecular weight between about 450 and about 650, said salt having an oleophilic residue containing at least about 16 carbon atoms.

15 10. The method of treating a hydrocarbon-containing system in its natural state in a well for the purpose of inhibiting corrosion by aqueous carbonic acid of well metal parts, said system comprising a non-oxidizing gas phase, a liquefied  
20 normally gaseous hydrocarbon phase and a minor amount of aqueous carbonic acid, which system in a state of agitated flow under a pressure of between about fifteen and seven thousand pounds per square inch absolute, comes in contact with  
25 corrodible well parts, which method includes the step of mixing with said system an amount of below approximately one weight per cent and above approximately 0.0001 weight per cent of the liquid hydrocarbon phase contacted, of an oil-  
30 soluble sodium petroleum mahogany sulfonate salt having a molecular weight between about 450 and about 650, said salt having an oleophilic residue containing at least about 16 carbon atoms.

11. The method of treating a hydrocarbon containing system in its natural state in a well for the purpose of inhibiting corrosion by aqueous carbonic acid of well metal parts, said system comprising a non-oxidizing gas phase, a liquefied normally gaseous hydrocarbon phase and a minor amount of aqueous carbonic acid, which system in a state of agitated flow under a pressure of between about fifteen and about seven thousand pounds per square inch absolute, comes in contact with corrodible well parts, which method includes the step of mixing with said system an amount of below approximately one weight per cent and above approximately 0.0001 weight per cent of an oil-soluble salt of an organic sulfonic acid having a molecular weight between about 450 and about 380, said salt having an oleophilic residue containing at least about 16 carbon atoms.

AARON WACHTER.  
WILFRID W. NEWSCHWANDER.

#### REFERENCES CITED

The following references are of record in the file of this patent:

UNITED STATES PATENTS

| Number    | Name            | Date           |
|-----------|-----------------|----------------|
| 1,630,101 | Wilkin          | May 24, 1927   |
| 1,878,468 | Covell          | Sept. 20, 1932 |
| 1,966,711 | De Groot et al. | July 17, 1934  |
| 2,453,881 | Viles et al.    | Nov. 16, 1948  |
| 2,453,882 | Viles et al.    | Nov. 16, 1948  |
| 2,461,359 | Viles et al.    | Feb. 8, 1949   |
| 2,466,517 | Blair et al.    | Apr. 5, 1949   |
| 2,466,530 | Blair et al.    | Apr. 5, 1949   |